

## UNITED STATES PATENT OFFICE

2,345,296

## LIQUID FUEL COMPOSITION

Walter A. Schulze and Joseph Preston Lyon, Jr.,  
Bartlesville, Okla., assignors to Phillips Petroleum Company, a corporation of Delaware

No Drawing. Application April 4, 1940,  
Serial No. 327,912

10 Claims. (Cl. 44—69)

This invention relates to a liquid hydrocarbon motor fuel composition, and to the method of preparing said composition. More specifically, this invention relates to the preparation of special hydrocarbon motor fuels containing tetraethyl lead in stable solution therein.

There are certain types of motor fuels such as high-octane aviation gasolines which are manufactured and blended according to specifications so strict that the selection of suitable components for blending is limited to synthetic or naturally occurring substantially pure hydrocarbons. Such blends must have high octane rating, because the tetraethyl lead content is limited, and accordingly, the hydrocarbon constituents of the blend must have an excellent response to addition of antiknock. Further, the olefinic or other unsaturated hydrocarbon content of the fuels must be almost nil, of the order of less than one per cent in order that the fuels be substantially free of gum and of susceptibility to gum formation. Also the absence of olefinic hydrocarbons is desirable because olefins contribute to excessive engine cylinder temperatures during combustion and are not very responsive to lead-alkyl antiknock compounds.

Such fuels are satisfactorily blended only from natural or synthetic, high-octane aliphatic or cyclic paraffin hydrocarbons although certain carefully selected aromatic compounds such as toluene may be used in some instances. The resulting blends of practically pure saturated hydrocarbons are substantially non-gum-forming and have an adequate response to the lead-alkyl antiknock. From the standpoint of storage stability, the outstanding possibility of deterioration of such a fuel in storage is the loss of octane number caused by loss of antiknock compound by precipitation from the fuel, and such deterioration is the subject of this invention.

It is an object of this invention to stabilize aviation gasolines which do not contain substantial amounts of highly unsaturated, gum-forming hydrocarbons such as olefins and diolefins and the like, and which contain an antiknock.

Another object of this invention is to provide a stable solution of tetraethyl lead in special motor fuels, composed of substantially non-gum-forming saturated hydrocarbons with olefinic content of less than one per cent, which have a tendency to deposit the antiknock as insoluble residues.

A further object of this invention is to prevent the separation or precipitation of lead-alkyl antiknock compounds from substantially

non-gum-forming hydrocarbon motor fuels which have a measurable tendency to precipitate said antiknock compounds and thereby lose the antiknock effect.

5 Other objects and advantages will become apparent from the following disclosure and discussion.

In the manufacture of very high octane motor fuels, such as 80 to 100 octane number aviation 10 gasolines, because of the limitation on tetraethyl lead addition the procedure usually includes the manufacture of synthetic isoparaffins. For example, such manufacture may include the polymerization of isobutylene to form isoctenes, followed by hydrogenation of the polymers to form isoctanes, with less than one per cent residual unsaturation.

These synthetic hydrocarbon fuels having an octane number of 90 to 100 may then be blended 20 with suitable saturated hydrocarbon stocks to meet the specifications governing volatility and vapor pressure. To such a blend is then added a quantity of an antiknock agent such as tetraethyl lead calculated to result in an octane number within the desired range.

The gasoline stocks which are suitable for use in such blends are carefully selected and are usually limited to saturated hydrocarbon liquids such as light straight-run naphthas which may 30 contain cyclo-paraffins and suitable fractions of natural gasolines which are predominantly aliphatic in nature, although certain non-gum-forming aromatic hydrocarbons such as toluene may be used, providing such use does not infringe any specifications for the fuel. The selection of such stocks, mainly pure hydrocarbons, with only negligible amounts of unsaturates and other impurities, is necessary because the finished blends must meet very stringent specifications regarding 35 acid heat tests, gum content and gum formation in storage.

The purity and inherent stability of fuels prepared by the above-outlined procedure, or the various possible modifications, is well illustrated 45 by the following abstract of U. S. Army Specifications No. 2-92-A. "The fuel must yield less than 6 milligrams of residue per 100 cubic centimeters, after evaporation of a portion of a 200 cubic centimeter sample which has been heated at 210° F. in contact with 35 square inches of steel surface for 5 hours under 100 pounds per square inch oxygen pressure." A fuel passing 50 such a test must certainly be judged substantially gum-free and non-gum-forming.

We have found that such fuels in spite of

purity, selected composition and inherent stability often exhibit a serious degradation; that is, the finished fuels containing an antidetonating agent such as tetraethyl lead often show a tendency to suffer the precipitation of insoluble residues from the tetraethyl lead under certain storage or test conditions such as the exposure to heat, oxygen and steel. On the other hand, the same fuels, before the addition of such an antidetonating agent, substantially lack the tendency to form gums, and do not contain appreciable quantities of olefins or diolefins or the like which ordinarily cause, or contribute to the formation of gum.

We have now discovered that the precipitation of lead compounds from liquid fuels of the type described which have a tendency to cause or to allow said precipitation may be prevented by the addition to the leaded fuel of small amounts of an efficient anti-oxidant, or gum-inhibitor, such as are available in commercial form to the industry and such as have been used heretofore only in fuels containing gum-forming hydrocarbons. The function of the inhibitor is, in the light of the foregoing description, not to prevent gum formation, since the hydrocarbon liquids of our composition are substantially non-gum-forming. In some manner, which is not precisely known to us, these added compounds are able either to maintain in their original form the solvents for the antidetonant or to stabilize directly the antidetonant compound and prevent its deterioration or chemical change.

The amount of inhibitor or anti-oxidant which we find effective in our composition is extremely small, being of the order of about 1 to 4 or more pounds of inhibitor per 1000 barrels of gasoline or in other terms between about 0.0001 and 0.002 per cent by weight of the fuel. These quantities are based on the use of anti-oxidants approximately as effective as monobenzyl-para-aminophenol, a widely used gum inhibitor. With less efficient anti-oxidants larger quantities may be required. The addition of the preferred quantity of anti-oxidant produces no deleterious effect on the fuel since other qualities are unimpaired. Since it is common commercial practice to purchase and use said inhibitors as solutions of varying concentrations in suitable solvents, it should be stated for the purpose of clarity that these preferred quantities are exclusive of the weight of such solvents or other material of like nature.

The means of adding the anti-oxidant to the liquid fuel may be any conventional method known to the industry, and the time of addition is generally just before or just after the addition of the tetraethyl lead composition, as may be convenient or desirable. After the fuel is thus blended, it is found that the conditions which would formerly cause precipitation of lead compounds in the uninhibited fuel no longer do so. Thus, exposure to the conditions of the previously mentioned gum test (U. S. Army No. 2-92-A) no longer causes any precipitation of insoluble lead compounds from the gasoline.

The following examples of the efficacy of our composition are included here, not as limiting our invention, but to illustrate some of the possible benefits. Many other analogous modifications and uses of our process will be obvious to those skilled in this art.

Components and finished blends of aviation gasoline were prepared and heated to 210° F. in a glass-lined bomb under 100 pounds per square inch oxygen pressure in contact with steel surface

for 5 hours. The following observations were made:

|    | Fuel                                                                        | Inhibitor                                                                   | Observations                           |
|----|-----------------------------------------------------------------------------|-----------------------------------------------------------------------------|----------------------------------------|
| 5  | Isooctane base+2 cc.<br>TEL/gallon.                                         | None                                                                        | Lead precipitate (decreased oct. No.). |
|    | Isooctane base+2 cc.<br>TEL/gallon.                                         | 0.0015% monobenzyl-para-amino-phenol.                                       | No precipitate.                        |
| 10 | 100 octane fuel (with<br>3 cc. TEL/gallon).                                 | None                                                                        | Lead precipitate (decreased oct. No.). |
|    | 100 octane fuel (with<br>3 cc. TEL/gallon).                                 | 0.0012% monobenzyl-para-amino-phenol.                                       | No precipitate.                        |
|    | 100 octane fuel (with<br>3 cc. TEL/gallon.)                                 | 0.008% Dupont No.<br>14 anti-oxidant (iso-<br>butyl-p-amino-<br>phenol).    | Do.                                    |
| 15 | Isooctane base+20%<br>pentane-free natural<br>gasoline+3 cc.<br>TEL/gallon. | None                                                                        | Lead precipitate (decreased oct. No.). |
|    | Isooctane base+20%<br>pentane-free natural<br>gasoline+3 cc.<br>TEL/gallon. | 0.0015% Dupont No.<br>9 anti-oxidant (n-<br>butyl-p-aminopheno-<br>nol).    | No precipitate.                        |
| 20 | 100 octane fuel (with<br>3 cc. TEL/gallon).                                 | 0.0004% Dupont No.<br>14 anti-oxidant (iso-<br>butyl-p-aminopheno-<br>nol). | Do.                                    |

In order to measure any corresponding effect on lead content occurring with ordinary motor fuels containing cracked gasolines which range from 10 to 40 per cent or more in unsaturation, induction period tests were made on several typical fuels. These tests included placing the sample of gasoline in a glass-lined bomb under 100 pounds per square inch oxygen pressure and heating the bomb at 210° F. until there was a rapid absorption of oxygen by the sample. After the test, the gasoline samples were examined, and while there was in some cases a resinous organic deposit, there was no evidence of substantial precipitation of lead residues. The results of these tests indicate that in ordinary cracked gasoline there is only negligible tendency to precipitate the antidetonant compound, whereas, in the case of predominantly saturated and substantially non-gum-forming aviation gasolines, the lead-precipitating tendency is greatly magnified.

The inhibitors which we find most effective in our composition are monobenzyl-para-aminophenol and homologous substituted aminophenols such as are commercially available to the industry.

Further, we disclaim all benefits and previously disclosed effects of the use of said gum inhibitors for the prevention or reduction of gum formation in motor fuels containing large amounts of olefinic, diolefinic and other unsaturated gum-forming hydrocarbons and gum-forming impurities. We emphasize the fact that the fuels to which we add said inhibitors are of such character as to be classified as substantially non-gum-forming, and that the qualities and uses of our special fuel composition are sufficient to distinguish over ordinary gum-forming fuels containing gum inhibitors.

What we claim is:

1. An improved aviation gasoline having an octane number above 80, comprising essentially a non-gum-forming hydrocarbon fuel containing less than one per cent by volume of olefinic or diolefinic hydrocarbons, tetraethyl lead and an aminophenol of the group consisting of monobenzyl-para-aminophenol, isobutyl-para-aminophenol, and normal butyl-para-aminophenol in an amount equal to between about 0.0004 to 0.002 weight per cent of the fuel as essentially the sole added material tending to inhibit decomposition and precipitation of said tetraethyl lead.
2. The method of preventing the precipitation

of insoluble lead compounds which tend to precipitate from a blend of tetraethyl lead antidetonant in essentially non-gum-forming aviation gasolines containing less than one per cent by volume of olefinic or other unsaturated hydrocarbons, which comprises adding to such a gasoline a small amount of an aminophenol of the group consisting of mono-benzyl-para-aminophenol, isobutyl-para-aminophenol, and normal butyl-para-aminophenol as essentially the sole added material tending to prevent the precipitation of the antidetonant compound.

3. The method of stabilizing aviation gasolines having an octane number above 80 and composed of essentially non-gum-forming hydrocarbons, with an olefinic or other unsaturated hydrocarbon content of less than one per cent, and tetraethyl lead which comprises adding to such a gasoline between 0.0008 and 0.002 weight per cent of monobenzyl-para-aminophenol as essentially the sole added material tending to inhibit decomposition and precipitation of said tetraethyl lead, whereby the precipitation of oil-insoluble lead compounds is inhibited.

4. A motor fuel composition, comprising essentially hydrocarbons in the boiling range of motor fuel and of such a character as to be classified as substantially non-gum-forming, an antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material tending to inhibit said decomposition and precipitation of said antidetonant.

5. A motor fuel composition, comprising essentially hydrocarbons in the boiling range of motor fuel and of such a character as to be classified as substantially non-gum-forming, an antidetonant compound which tends to decompose and be precipitated when in admixture with such hydrocarbons under normal conditions of storage and handling of aviation motor fuel, and a small amount of monobenzyl-para-aminophenol as essentially the sole material tending to inhibit said decomposition and precipitation of said antidetonant.

6. A motor fuel composition, comprising essentially hydrocarbons in the boiling range of motor fuel and of such a character as to be classified as substantially non-gum-forming, tetraethyl lead which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, 60

and normal butyl-para-aminophenol as essentially the sole material tending to inhibit said decomposition and precipitation of said tetraethyl lead.

5 7. A motor fuel composition, comprising essentially hydrocarbons in the boiling range of motor fuel and of such a character as to be classified as substantially non-gum-forming, a lead-alkyl antidetonant compound which tends to decompose

10 and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material tending to inhibit said decomposition and precipitation of said antidetonant.

8. A motor fuel composition, consisting essentially of paraffin hydrocarbons in the boiling range of motor fuel and containing less than one per cent by volume of unsaturated hydrocarbons, a lead-alkyl antidetonant compound which tends to decompose and form precipitate when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

20 9. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

25 10. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

30 11. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

35 12. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

40 13. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

45 14. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

50 15. A motor fuel composition, comprising essentially hydrocarbons in the boiling range of motor fuel and of such a character as to be classified as substantially non-gum-forming, a lead-alkyl antidetonant compound which tends to decompose and be precipitated when in admixture with such hydrocarbons under normal conditions of storage and handling of aviation motor fuel, and a small amount of an aminophenol of the group consisting of monobenzyl-para-aminophenol, isobutyl-para-aminophenol, and normal butyl-para-aminophenol as essentially the sole material present tending to inhibit said decomposition and precipitation of said antidetonant.

WALTER A. SCHULZE,  
JOSEPH PRESTON LYON, JR.